

## UNITED STATES PATENT OFFICE

2,592,366

NONCAKING PHOTOGRAPHIC ACID  
FIXING POWDERS

Edwin S. Wiitala and Donald J. Kridel, Rochester, N. Y., assignors to Eastman Kodak Company, Rochester, N. Y., a corporation of New Jersey

No Drawing. Application February 9, 1951,  
Serial No. 210,283

9 Claims. (Cl. 95—88)

1

This invention relates to photographic fixing powders, and more particularly to an improved single-powder acid fixing powder composition which has substantially no tendency to cake while in a package and exposed to various atmospheric conditions.

Fixing compositions in powder form containing in addition to sodium thiosulfate, commonly called hypo, other substances such as salts of acetic acid, alum, etc., have been known for many years. Fixing solutions which are made by adding water to such powder compositions perform several functions in addition to fixing out the unexposed silver salts of the photographic emulsion. The acid in them neutralizes the developer carried over by films or prints and prevents the fixing bath from becoming alkaline. A hardening agent is often included in such formulas to harden the emulsion and protect it from mechanical injury during subsequent processing or from the slightly elevated temperature employed in drying. Sulfurization inhibitors are also added to prevent interaction between the acids and the thiosulfate. The hardening agent most commonly employed is alum i. e. potassium aluminum sulfate or ammonium aluminum sulfate. Many fixing powders of the acid hardening type in addition to hypo contain potassium alum as the hardener, an acetate, and sodium sulfite as the inhibiting agent.

Fixing baths containing such materials represent rather complex chemical systems in which certain factors must be accurately adjusted to give satisfactory results. Qualities of such fixing baths such as degree of hardening, hardening life, sludging and rate of sulfurization are all interdependent and are influenced by the amount of the various ingredients and the ratio of these amounts to each other. It is usually true that if an attempt is made to adjust the 40 bath for the optimum of a certain property, one or more of the other properties is sacrificed to some extent. Thus, for example, it is possible that if an attempt is made to secure the maximum degree of hardening, the rate of sulfurization or of sludging may be adversely affected. Consequently there are several features in present fixing compositions which should be bettered and the instant invention describes such an improvement.

Hardening life is defined as the amount of fixing which can be done during which the fixing bath retains a satisfactory degree of hardening. Hardening life may be measured by plotting the temperature at which the gelatin film begins to melt against the amount of a developer which has been added to the fixing bath. This closely

2

parallels the actual conditions under which the bath is employed. The type of curve obtained with the usual fixing bath is one which quickly rises to a maximum and then rapidly falls as more developer is added. When a moderate amount of developer has been added the fixing bath will no longer harden satisfactorily.

In Patent 1,930,140 of October 10, 1933, a successful method of increasing the hardening life 10 of a fixing bath without adversely affecting any of its other qualities is described. Fixing baths made in accordance with the procedure of Patent 1,930,140 will maintain satisfactorily hardening over a much wider range, in other words, they 15 will still harden satisfactorily when a large amount of developer has been added to them.

As described in the patent, the acid fixing powders contain a substance capable of furnishing acid components to the bath, such as an alkali metal acetate and boric acid. Satisfactory 20 substances which furnish the acetate ion are sodium acetate and sodium diacetate though other acetates may be employed. Sodium citrate and sodium tartrate may also be employed instead of sodium acetate. The boric acid is added either as such or is supplied by borax and acetic acid in solution. A small amount of boric acid is, therefore, present in the fixing bath simultaneously with the acetate ion. Alum is also 25 present in the bath composition.

These fixing baths will give a greatly increased 30 hardening life. They will still harden satisfactorily when from three to four times as much developer is carried over as will render an ordinary bath unfit for further use.

While these fixing baths operate very satisfactorily, the powders, to which water is added to make up the bath, are sold in a packaged form in which they are quite uniformly mixed together. These powders, per se, introduce another difficulty in the problem of obtaining effective fixing 35 operations.

It was found at elevated temperatures i. e. 100° F. and above that the powders made in accordance with Patent 1,930,140 tended to cake 40 together and hence cause difficulty in removing a desired amount from the package.

This caking appears to be a result of moisture liberation from the alum and other powders at 45 such elevated temperatures. On cooling, the liberated moisture is in sufficient amount to cause fusion of the powder, possibly as hydrates of the hypo.

An object, therefore, of the present invention 50 is to provide an acid fixing powder having improved hardening characteristics as compared to those disclosed in the prior art.

Another object of the invention is to provide an acid fixing powder having improved hardening characteristics without the tendency of caking at elevated temperatures.

In accordance with the invention these and other objects are attained by replacing boric acid in the acid fixing powders with boric anhydride. The boric anhydride may contain up to 15.0% by weight of free moisture and still be usable in our improved fixing bath. Our studies have indicated that boric anhydride has an advantageous desiccating action and also has the desirable property of remaining as a dry powder upon reacting with the amount of moisture present in the acid fixing powders, that moisture heretofore being the cause of caking. We have discovered that boric anhydride can be substituted in corrected amount of the boric acid in acid fixing powders, as mentioned above, without any apparent disadvantages. This substitution has the great advantage of virtually eliminating the caking of the fixing powder. When these powders are put in a water solution, the boric anhydride forms boric acid in the desired amount.

The following examples are illustrative of our improved acid fixing powder compositions:

*Example 1*

|                              | Grams |
|------------------------------|-------|
| Anhydrous sodium thiosulfate | 160   |
| Sodium sulfite               | 5     |
| Sodium bisulfite             | 5     |
| Boric anhydride              | 2.8   |
| Sodium acetate               | 22.5  |
| Ammonium alum                | 22.5  |

*Example 2*

|                  | Grams |
|------------------|-------|
| Hypo             | 300   |
| Sodium bisulfite | 12.5  |
| Potassium alum   | 15    |
| Sodium acetate   | 18    |
| Boric anhydride  | 2.8   |

In these formulas a portion or all of the sodium acetate may be replaced by equivalent amounts of sodium citrate or sodium tartrate acids. However, sodium acetate is preferred. The compositions in Examples 1 and 2 are put in solution in water to make up one liter of fixing bath. These fixing baths will give a greatly increased hardening life. They will still harden satisfactorily when from three to four times as much developer is carried over as will render many acid fixing baths unfit for further use.

The preferred range of concentration of the acetate ions is from 10 grams per liter to 40 grams per liter, and the amount of hardeners is not less than 5 grams and is preferably less than 30 grams per liter. Boric anhydride may be present in amounts up to 20 grams per liter. Only 56.3% of the boric acid content normally present in such baths is required as boric anhydride, due to the higher borate content in the anhydride.

*Comparative test*

A sample of acid fixing powder of the present invention shown in Example 2 and containing boric anhydride was compared with a sample of the powder shown in Example III of Patent 1,930,140 containing boric acid. In preparing the sample according to Example III of Patent 1,930,140, the sodium acetate crystals were replaced with an equivalent amount of anhydrous sodium acetate. After one day at 110° F. the acid fixing powder containing boric acid had caked considerably, while the boric anhydride acid fix

was perfectly free flowing. After one week at 110° F. the regular fixer was moderately caked and the other with the boric anhydride was free flowing. The solution rate of the boric anhydride fixer sample was comparable to the regular, if not better. It can be considered better in that no slowly soluble lumps are introduced into the solution as is the case with a caked material.

Our invention, therefore, supplies to the art a valuable improvement in the fixing powder field.

What we claim and desire to secure by Letters Patent of the United States of America is:

1. A non-caking acid fixing powder composition containing sodium thiosulfate, an alkali sulfite, a hardening agent, boric anhydride, and a salt of a solid organic acid selected from the group consisting of acetic, citric and tartaric acids.

2. A noncaking acid fixing powder composition containing sodium thiosulfate, an alkali bisulfite, a hardening agent, boric anhydride, and a salt of a solid organic acid selected from the group consisting of acetic, citric and tartaric acids.

25 3. A non-caking acid fixing powder composition containing sodium thiosulfate, an alkali sulfite, a hardening agent, boric anhydride, and an alkali metal acetate.

4. A non-caking acid fixing powder composition containing sodium thiosulfate, sodium sulfite, alum, boric anhydride and sodium acetate.

30 5. A non-caking acid fixing powder composition containing sodium thiosulfate, sodium sulfite, alum, boric anhydride and sodium citrate.

6. A substantially non-caking powdered material capable, when dissolved, of constituting an acid hardening fixing bath comprising:

|                              | Grams |
|------------------------------|-------|
| Anhydrous sodium thiosulfate | 160   |
| Sodium sulfite               | 5     |
| Sodium bisulfite             | 5     |
| Boric anhydride              | 2.8   |
| Sodium acetate               | 22.5  |
| Ammonium alum                | 22.5  |

7. A substantially non-caking powdered material capable, when dissolved, of constituting an acid hardening fixing bath comprising:

|                              | Grams |
|------------------------------|-------|
| Anhydrous sodium thiosulfate | 300   |
| Sodium bisulfite             | 12.5  |
| Potassium alum               | 15.0  |
| Sodium acetate               | 18.0  |
| Boric anhydride              | 2.8   |

8. A substantially non-caking powdered material capable, when dissolved, of constituting an acid hardening fixing bath comprising:

|                              | Grams |
|------------------------------|-------|
| Anhydrous sodium thiosulfate | 300   |
| Sodium bisulfite             | 12.5  |
| Potassium alum               | 15.0  |
| Sodium citrate               | 18.0  |
| Boric anhydride              | 2.8   |

9. A substantially non-caking powdered material capable, when dissolved, of constituting an acid hardening fixing bath comprising:

|                              | Grams |
|------------------------------|-------|
| Anhydrous sodium thiosulfate | 300   |
| Sodium bisulfite             | 12.5  |
| Potassium alum               | 15.0  |
| Sodium tartrate              | 18.0  |
| Boric anhydride              | 2.8   |

EDWIN S. WIITALA.  
DONALD J. KRIDEL.